

## 1

3,124,411

METHOD FOR DYEING TEXTILE MATERIALS  
WITH VAT DYES

Gilbert S. Panson and Carol E. Weill, Livingston, N.J.,  
assignors to Metal Hydrides Incorporated, Beverly,  
Mass., a corporation of Massachusetts  
No Drawing. Filed July 17, 1961, Ser. No. 124,373  
6 Claims. (Cl. 8—34)

This invention relates to dyeing textile materials with  
vat dyes.

Textile materials, such as cotton fabrics, usually are  
dyed by padding a vat dye on to the fabric, squeezing  
out the excess, and then passing the dye impregnated  
fabric through an aqueous bath containing sodium hy-  
droxide, sodium hydrosulfite and sodium chloride. The  
reducing liquor reduces the dye and converts it to the  
water soluble sodium leuco form, the presence of the salt  
shifting the equilibrium of the reduced dye from the solu-  
tion to the fabric. The cloth then is removed from the  
bath and the dye oxidized to give a level dyeing of de-  
sired shade. This procedure requires the use of as much  
as 5 to 40 fold excess of hydrosulfite over the stoichio-  
metric requirement since the hydrosulfite is very unstable  
under the conditions of air oxidation present in dyeing  
and the high temperatures used in the dyeing operation.

It has been proposed heretofore that an alkali metal  
bisulfite, such as sodium bisulfite, can be converted to  
alkali metal hydrosulfite in an aqueous medium by the  
addition of an alkali metal borohydride, such as sodium  
or potassium borohydride. Thereafter, an alkali metal  
hydroxide may be added and the resulting alkaline solution  
may be used for reducing vat dyes and for dyeing  
textile fabrics by immersing the textile fabric in the al-  
kaline hydrosulfite solution. This procedure does not  
solve the instability problem of the hydrosulfite and re-  
quires the substantial absence of alkaline metal hydroxide  
during the reaction between the alkali metal bisulfite and  
alkali metal borohydride.

The present invention is based upon the discovery that  
if a textile fabric is impregnated with a mixture of a  
vat dye and an alkali metal bisulfite and the thus im-  
pregnated fabric is passed through a reducing liquor con-  
sisting of an aqueous solution of an alkali metal hy-  
droxide and an alkali metal borohydride having a pH  
between about 9.5 and 13, the vat dye is reduced and  
converted to its water soluble alkali leuco form. Thus,  
in accordance with the method of the present invention,  
a mixture of a vat dye and an alkali metal bisulfite, such  
as sodium bisulfite, in the form of an aqueous dispersion  
is padded on to the textile fabric, the excess being  
squeezed out. The thus impregnated fabric then is passed  
through an aqueous reducing solution consisting essen-  
tially of an alkali metal hydroxide, such as sodium hy-  
droxide, an alkali metal borohydride, such as sodium or  
potassium borohydride, and a salt, such as sodium chlo-  
ride. The fabric then is removed from the reducing  
solution and subjected to an oxidizing operation.

Since the composition of the various vat dyes varies, the  
amounts of alkali metal bisulfite and alkali metal bor-  
ohydride required in the practice of the invention will  
vary. In general, about 4 to 400 parts by weight of  
alkali metal bisulfite and about 0.2 to 20 parts by weight  
of alkali metal borohydride per 100 parts by weight of  
vat dye may be used. The use of greater amounts of  
bisulfite and borohydride are not harmful. It will be  
understood that in a continuous dyeing operation, the  
concentration of alkali metal hydroxide, alkali metal  
borohydride, and salt in the reducing bath must be main-  
tained sufficiently high and, preferably, substantially con-  
stant to effect the desired reduction and obtain level dye-  
ing.

## 2

The amount of sodium hydroxide required in the re-  
ducing bath varies with the class of vat dye used and can  
be determined from the booklets published by the dye  
manufacturer. Each dye works best at a certain sodium  
hydroxide level. Sufficient sodium hydroxide in ex-  
cess of the amount required to convert the dye to its  
alkali leuco form must be present to stabilize the bath.

In some instances in commercial operation it is desira-  
ble to dry the impregnated fabric before immersion in  
the reducing bath. Cloth impregnated with vat dye and  
sodium bisulfite in accordance with the invention can be  
dried at 110° C. for 1 to 2 hours and then immersed  
in the reducing bath and obtain the desired shade. This  
indicates the great stability of the mixture of bisulfite  
and vat dye.

Reduction of the dye to the sodium leuco and ex-  
haustion of the dye in to the fabric is dependent upon the  
temperature of the bath and the time of contact. At  
high temperatures, such as 80° C. and higher, the con-  
tact time is less than 10 seconds which makes the inven-  
tion particularly useful for continuous dyeing, such as  
in the Williams unit. At lower temperatures, longer con-  
tact times are needed to insure full reduction and pene-  
tration of the dye. The latter conditions are more useful  
in the Beck dyeing operations or package dyeing opera-  
tions where longer contact times are needed.

The mixture of alkali metal bisulfite and vat dye used  
in the practice of the invention is completely stable and  
can be stored for long periods of time. The aqueous sol-  
ution of alkali metal hydroxide and alkali metal borohy-  
dride is available in concentrations which also are ex-  
tremely stable even at high temperatures for long periods  
of time. When the fabric impregnated with the mix-  
ture of alkali metal bisulfite and vat dye is passed into  
the reducing solution, the vat dye is reduced and con-  
verted to its water soluble alkali leuco form in a very  
few seconds. Consequently, the residence time required  
in the reducing bath is very short and there is very little  
opportunity for the side reaction of air oxidation to occur.  
This is of particular industrial significance because  
it makes possible vatting operations with substantially less  
reducing agent than has heretofore been required.

While we have described the use of the alkali metal  
borohydrides in the practice of the invention, the quater-  
nary ammonium borohydrides may be used in place  
thereof if desired. As illustrative of water soluble qua-  
ternary ammonium borohydrides we may mention the  
lower tetraalkyl ammonium borohydrides, such as tetra-  
methyl, tetraethyl, trimethyl ethyl, dimethyl diethyl am-  
monium borohydrides, as well as quaternary ammonium  
borohydrides responding to the formula  $R_x(CH_3)_yNBH_4$   
where R is a saturated or unsaturated straight chain  
aliphatic hydrocarbon radical containing about 7 to 21  
carbon atoms, x and y are integers from 1 to 3, and x  
plus y equals 4, such as tricapryl methyl ammonium  
borohydride, cetyl trimethyl ammonium borohydride, etc.

We have successfully used in the practice of the inven-  
tion many vat dyes selected from the various types com-  
monly used in commercial practice. As illustrative of  
such vat dyes we may mention anthraquinone type dyes,  
such as Mayvat Jade Green (C.I. #59,105), Carbanthrene  
Blue BCS (C.I. #69,825), Ponsul Brilliant Violet 4RN  
(C.I. #60,010), Ponsul Golden Orange 3G (C.I.  
#69,025), Indanthrene Golden Yellow RK (Vat Orange  
1, C.I. #59,105/6), Indanthrene Brilliant Orange RK  
(Vat Orange 3, C.I. #59,300), Amanthrene Golden  
Orange F (Vat Orange 9, C.I. #59,700), Indanthrene  
Orange RRT (Vat Orange 1, C.I. #59,705), and Indan-  
threne Dark Blue BO (Vat Blue 20, C.I. #59,800),  
Tinon Navy Blue RAF (Vat Blue 18, C.I. #59,815),  
Ahcovat Jade Green B (Vat Green 1, C.I. #59,825),  
Indanthrene Brilliant Violet 3B (Vat Violet 9, C.I.

#60,005), Cibanone Violet 4R (Vat Violet 1, C.I. #60,010); anthraquinone type dyes containing amino groups, such as Cibanone Black DRB (Vat Black 9, C.I. #65,230); dyes containing a heterocyclic nucleus fixed to a central vatting system, such as Indanthrene Red FBB (Vat Red 10, C.I. #67,000), Tinon Yellow GC (Vat Yellow 2, C.I. #67,300), Carbanthrene Red BN (Vat Red 35, C.I. #68,000), Cibanone Violet BNA (Vat Violet 13, C.I. #68,700), Indanthrene Brown RN (Vat Brown 3, C.I. #69,015), Indanthrene Red Brown 5 RF (Vat Brown 25, C.I. #69,020), Tinon Olive BF (Vat Green 3, C.I. #69,500), Tinon Olive SF (Vat Black 25, C.I. #69,525), Cibanone Blue GCDN (Vat Blue 14, C.I. #68,810), Ponsul Blue BF (Vat Blue 6, C.I. #69,825), Indanthrene Khaki GG (Vat Green 8, C.I. #71,050); indigo and its derivatives and homologues, such as Cibanone Blue 2BGD (Vat Blue 5, C.I. #73,065); thio-indigo and its derivatives and homologues, such as Hostavat Brilliant Pink R (Vat Red 1, C.I. #73,360), Indanthrene Printing Violet 6R (Vat Violet 3, C.I. #73,395); phthalocyanine dyes, such as Algol Brilliant Blue 4G (Vat Blue 29, C.I. #74,140).

The invention is illustrated further by the following specific examples, the results of which are shown in the following tables. In all of these examples level dyeings to the shade specified by the dye manufacturer were obtained. In these tables the term "reduced" indicates proper sodium leuco was formed and samples of cloth dyed gave the color and shade indicated by the dye manufacturer.

In the following tables the following formulations were used as standard unless otherwise indicated in the table.

#### PAD BATH

4.0 grams of vat dye (as a single paste) was diluted with 125.0 grams of water and 8.3 grams of sodium bisulfite was stirred into the diluted paste. Variable amounts of water or dye can be used depending upon the final shade desired. Cotton cloth was immersed in this mixture and then passed through squeeze rolls to remove the excess.

#### REDUCING BATH

The standard reducing bath contained 0.2 gram of sodium hydroxide, 0.4 gram of sodium borohydride, 20 grams of sodium chloride and 250 grams of water. The bath was heated to 80° C. The cloth from the squeeze rolls was passed into the reducing bath where reduction took place rapidly. The cloth then was removed and subjected to a conventional oxidizing operation.

Table I

| Example | Dye Used                     | Temp. (° C.) | pH    | Contact Time | Comment            |
|---------|------------------------------|--------------|-------|--------------|--------------------|
| 1.....  | Vat Red 1, (C.I. #73,360)    | 80           | 11.3  | 5 sec....    | Reduced.           |
| 2.....  | Vat Red 29, (C.I. #71,140)   | 80           | 11.3  | 5 sec....    | Do.                |
| 3.....  | Vat Orange 5, (C.I. #73,335) | 80           | 11.3  | 5 sec....    | Do.                |
| 4.....  | Vat Yellow 2, (C.I. #67,300) | 80           | 11.3  | 5 sec....    | Do.                |
| 5.....  | Vat Yellow 4, (C.I. #59,100) | 80           | 11.3  | 5 sec....    | Do.                |
| 6.....  | Vat Green 1, (C.I. #59,825)  | 24           | 11.45 | 5 min....    | Partially reduced. |
| 7.....  | do.....                      | 80           | 11.3  | 5 sec....    | Reduced.           |
| 8.....  | do.....                      | Boil         | 11.25 | 1 sec....    | Do.                |
| 9.....  | Vat Blue 5, (C.I. #73,065)   | 80           | 11.3  | 5 sec....    | Do.                |
| 10..... | Vat Blue 6, (C.I. #69,825)   | 80           | 11.3  | 1 sec....    | Do.                |
| 11..... | Vat Blue 20, (C.I. #59,800)  | 80           | 11.3  | 5 sec....    | Do.                |
| 12..... | Vat Blue 43, (C.I. #53,630)  | 80           | 11.3  | 5 sec....    | Do.                |
| 13..... | Vat Violet 3, (C.I. #73,396) | 80           | 11.3  | 5 sec....    | Do.                |
| 14..... | Vat Black 25, (C.I. #69,525) | 80           | 11.3  | 5 sec....    | Do.                |

The pH indicated is that at the temperature shown in the table before immersing the impregnated cloth.

Table II

5 This table illustrates the effect of the ratio of dye to sodium bisulfite, the dye used being Vat Green 1 (C.I. #73,360).

| Example | Dye in grams | NaHSO <sub>3</sub> in grams | Ratio of dye to NaHSO <sub>3</sub> | pH   | Comment               |
|---------|--------------|-----------------------------|------------------------------------|------|-----------------------|
| 19..... | 15.0         | 0.5                         | 30.0                               | 11.3 | Reduction incomplete. |
| 20..... | 20.0         | 1.0                         | 20.0                               | 11.3 | Reduced.              |
| 21..... | 10.0         | 1.0                         | 10.0                               | 11.3 | Do.                   |
| 22..... | 15.0         | 8.3                         | 1.8                                | 11.3 | Do.                   |
| 23..... | 4.0          | 8.3                         | 0.48                               | 11.3 | Do.                   |
| 24..... | 4.0          | 12.0                        | 0.33                               | 11.3 | Do.                   |

The pH is that at the temperature of 80° C. before immersing the impregnated cloth.

Table III

25 This table illustrates the effect of the ratio of sodium bisulfite to sodium borohydride, the dye used being Vat Green 1 (C.I. #73,360).

| Example | NaHSO <sub>3</sub> in grams | NaBH <sub>4</sub> in grams | Ratio of NaHSO <sub>3</sub> to NaBH <sub>4</sub> | pH              | Comment  |
|---------|-----------------------------|----------------------------|--------------------------------------------------|-----------------|----------|
| 25..... | 8.3                         | 0.4                        | 20.75                                            | 11.3            | Reduced. |
| 26..... | 12.0                        | 0.1                        | 120.0                                            | 9.6             | Do.      |
| 27..... | 0.5                         | 0.4                        | 1.25                                             | 11.9            | Do.      |
| 28..... | 8.3                         | 8.7                        | 0.95                                             | 12 <sup>+</sup> | Do.      |

35 The pH indicated is that at a temperature of 80° C. before immersing the impregnated cloth.

We claim:

1. In a method for continuously dyeing textile materials with vat dyes which involves padding the textile material with an aqueous dispersion of the vat dye and passing the dye impregnated textile material through an aqueous solution of a vat dye reducing agent, the improvement wherein the textile material is impregnated with a mixture of the vat dye and an alkali metal bisulfite and the textile material impregnated with the vat dye and bisulfite is passed through an aqueous solution of a borohydride and an alkali metal hydroxide having a pH between about 9.5 and 13, said borohydride being selected from the group consisting of alkali metal borohydrides and quaternary ammonium borohydrides.

2. The method as claimed by claim 1 wherein the borohydride is an alkali metal borohydride.

3. The method as claimed by claim 1 wherein the borohydride is a water soluble quaternary ammonium borohydride.

4. The method as claimed by claim 1 wherein the alkali metal bisulfite is sodium bisulfite.

5. The method as claimed by claim 2 wherein the alkali metal borohydride is sodium borohydride.

6. The method as claimed by claim 4 wherein the borohydride is sodium borohydride.

#### References Cited in the file of this patent

#### UNITED STATES PATENTS

2,745,788 Frohnsdorff \_\_\_\_\_ May 15, 1956  
2,991,152 Goerrig et al. \_\_\_\_\_ July 4, 1961

#### FOREIGN PATENTS

70 1,036,228 Germany \_\_\_\_\_ Aug. 14, 1958

#### OTHER REFERENCES

Vickerstaff, The Physical Chemistry of Dyeing, pages 280-283, pub. by Interscience Pub. Inc., N.Y.C., 1954.